

1

3,454,424

PROCESS FOR MAKING PHOTOGRAPHIC FILMS  
Rudolf Schneider, Neu-Isenburg, Germany, assignor to  
E. I. du Pont de Nemours and Company, Wilmington,  
Del., a corporation of Delaware  
No Drawing. Filed June 21, 1966, Ser. No. 559,082  
Claims priority, application Germany, July 30, 1965,

A 49,885

Int. Cl. B32b 32/12, 27/06; G03c 1/78

U.S. Cl. 117—145

5 Claims 10

## ABSTRACT OF THE DISCLOSURE

A process for making dimensionally stable cellulose organic monocarboxylic acid ester film base by applying to the base a solution of a copolymer of one mole of maleic anhydride with one mole of a different addition polymerizable ethylenically unsaturated monomer having a vinyl group not substituted on the  $\alpha$ -carbon atom of said group in a solvent blend of 50% to 80% ethyl acetate and 50% to 20% isopropanol, by weight. Vinyl acetate and vinyl chloroacetate and cellulose triacetate and cellulose acetate/butyrate are useful materials.

This invention pertains to a process for making dimensionally stable photographic films having a support composed of organic cellulose esters.

It is known that photographic films undergo dimensional changes under the influence of varying atmospheric conditions. Dimensional variations also occur in processing photographic films, even under constant atmospheric conditions. Under the effects, usually rather prolonged, of aqueous and sometimes strongly alkaline processing baths the photographic film first swells, only to shrink again during the subsequent drying process. The dimensional changes involved here are irreversible, i.e. the initial dimensions of the photographic film are not regained but instead permanent dimensional changes occur. For example, it can usually be observed that photographic films have shrunk, as compared with their initial state at the instant of exposure, after the developing and drying processes.

For many types of photographic films, especially in copying methods, aerial photography and others, dimensional stability of the photographic film is important.

The film base itself is the controlling factor for the dimensional stability of the coated photographic films. The photosensitive layer, however, has some influence, especially on dimensional changes which occur during processing of the coated film. As applicants have been able to demonstrate, this is particularly true of the type of film supporting treatment, the solvent employed in applying the film support having in particular a substantial influence. Efforts have been made to improve dimensional stability of photographic films by using strongly hydrophobic plastic film base. In this respect, the best dimensional stability is obtained with hydrophobic film base made from polyesters of terephthalic acid with ethylene glycol, and by polystyrene or polycarbonate films.

Nevertheless, it is known that dimensional stability of such hydrophobic film bases can be implemented only if they are coated with photosensitive emulsions in which at least a part of the gelatin has been replaced by synthetic plastics. Such a replacement of gelatin sometimes has, on the other hand, a highly unfavorable effect on the photographic properties of the emulsions, so that for the sake of photographic quality of the product the ultimate choice is to accept decreased dimensional stability as compared with the uncoated foil. Because of this and other disadvantages, such as difficulties in preparation and in

2

subbing the film support, film bases composed of organic cellulose esters, e.g. cellulose acetate, cellulose propionate, cellulose acetate/propionate, and cellulose acetate/butyrate, and especially cellulose triacetate, still constitute commercially useful bases for many purposes.

A requirement which organic cellulose ester films are still unable to meet fully, in spite of their excellent mechanical properties, is the extraordinary demand imposed by modern copying techniques on dimensional stability of film supports. For example, photographic film having a cellulose triacetate base undergoes, during the various stages of preparation and processing under constant atmospheric conditions changes in length as set forth in Table I below, wherein a negative sign means that the film has shrunk while a positive sign indicates that the finished processed film has increased in length.

TABLE I

|    |                                                                                                                       | Percent change in film length |
|----|-----------------------------------------------------------------------------------------------------------------------|-------------------------------|
| 20 | Film preparation stage:                                                                                               | caused by processing          |
|    | Cellulose triacetate film support not substrate treated                                                               | +0.030                        |
|    | Cellulose triacetate film support treated with a substrate solution from the prior art, containing gelatin            | -0.070                        |
|    | Cellulose triacetate film support, coated as in the prior art and coated with a photosensitive silver halide emulsion | -0.100                        |

As may be seen from Table I, only the substrate treatment by itself causes a change of 0.100% in dimensional stability whereas application of the photosensitive layer merely causes an additional 0.030% of shrinkage.

Now it has been found that this decrease in dimensional stability to processing, caused by the substrate treatment in organic cellulose ester film bases can be prevented by using as subbing solution for the film support a solvent blend of ethyl acetate and isopropanol, and as the adhesive copolymers of maleic anhydride with other polymerizable monomers containing vinyl groups which are not substituted on the  $\alpha$ -carbon atom of the vinyl group. Suitable such copolymers are disclosed in German Patent 1,040,898.

A photosensitive film, containing a subbing layer, prepared from maleic anhydride copolymer and the above mentioned solvents undergoes substantially no dimensional change in processing baths and is characterized by excellent dimensional stability. Table II shows the improvement in dimensional stability to processing in finished, emulsion-coated films obtained in accordance with this invention.

TABLE II

|                         |                                                                                                                 | Percent change in film length, |
|-------------------------|-----------------------------------------------------------------------------------------------------------------|--------------------------------|
| Film preparation stage: | caused by processing                                                                                            |                                |
| 55                      | Cellulose triacetate film support, untreated                                                                    | +0.30                          |
|                         | Cellulose triacetate film support, prepared for substrate in accordance with this invention                     | +0.025                         |
| 60                      | Cellulose triacetate film support, prepared for substrate in accordance with this invention and emulsion-coated | -0.005                         |

Thus it is possible, according to this invention, to effect an improvement in dimensional stability to processing in photographic films having an organic cellulose ester film support, especially cellulose triacetate, that the dimensional change occurring after processing is less than  $\pm 0.01\%$ .

In addition to their beneficial effect on dimensional stability to processing, substrate layers made in accordance with this invention are excellent adhesive agents between the film support and the photosensitive emulsion, and in

other respects also they meet all requirements which these layers must satisfy.

The optimum adhesive effect and dimensional stability is attained in general when use is made of a solvent blend of 50-80% ethyl acetate and 50-20% isopropanol.

It is completely unexpected and in no way obvious to one skilled in the art that by using the disclosed maleic anhydride copolymers and ethyl acetate and isopropanol as the solvent blend, one can obtain an improvement in dimensional stability to processing in the finished film product. That this result is surprising is evidenced by the fact that if ethyl acetate and/or isopropanol are replaced by other solvents, e.g., acetone and/or methanol, customarily used for coating copolymer subbing layers in making photographic film base, dimensional stability is seriously impaired.

Corresponding comparative tests gave the results set forth in the following table:

bases made of organic cellulose monocarboxylic acid esters, e.g. fatty acids of 2-4 carbon atoms, can be improved. Suitable esters include cellulose triacetate, cellulose acetopropionate, and cellulose acetobutyrate which can be so much improved that they are far superior in this respect to substrate treated cellulose ester film supports of the prior art and sometimes even attain the quality of known hydrophobic polymer film supports e.g. polyethylene terephthalate supports.

The following representative example is intended to explain the process in greater detail. The parts are by weight.

#### Example

A cellulose triacetate foil, 140 microns thick, consisting of 100 parts cellulose triacetate (acetic acid content 61.0%) and 15 parts triphenyl phosphate, prepared from a solution of these substances in methylene chloride:

TABLE III

| Film base                                                                                                    | Percent change in length by processing a film made by applying a substrate solution containing the solvent blends— |                                                              |                                 |                                              |                                                            |
|--------------------------------------------------------------------------------------------------------------|--------------------------------------------------------------------------------------------------------------------|--------------------------------------------------------------|---------------------------------|----------------------------------------------|------------------------------------------------------------|
|                                                                                                              | 50-80% EtOAc,<br>50-20%<br>Me <sub>2</sub> CHOH                                                                    | 50-80% Me <sub>2</sub> CO,<br>50-20%<br>Me <sub>2</sub> CHOH | 50-80% EtOAc,<br>50-20%<br>MeOH | 50-80% Me <sub>2</sub> CO,<br>50-20%<br>MeOH | 25-40% EtOAc,<br>25-40% Me <sub>2</sub> CO,<br>50-20% MeOH |
| Cellulose triacetate film support not substrate treated                                                      |                                                                                                                    |                                                              | +0.030                          |                                              |                                                            |
| Cellulose triacetate film base substrate treated with solvent blends                                         | +0.025                                                                                                             | -0.020                                                       | +0.005                          | -0.050                                       | -0.025                                                     |
| Cellulose triacetate film base substrate treatment as indicated coated with a gelatin-silver halide emulsion | -0.005                                                                                                             | -0.050                                                       | -0.025                          | -0.080                                       | -0.055                                                     |

As may be determined from Table III, wherein Me is methyl, Et is ethyl and Ac is CH<sub>3</sub>COO, the improvement in dimensional stability to processing is attained only when the maleic anhydride copolymer is applied from a solvent blend, e.g. ethyl acetate and isopropanol, in accordance with this invention.

It should be recognized that it is impossible to prepare stable gelatin-containing substrate solutions in absence of water, using only ethyl acetate and isopropanol, so that the observation underlying the present invention could not have been determined from a simple conversion of a classical substrate preparation method to the basis of using gelatin.

Suitable copolymers for carrying out the process as disclosed are chiefly those made from maleic anhydride and vinyl acetate, the two components being employed preferably in approximately equivalent quantities. There are, however, other copolymers, e.g. those made from maleic anhydride and vinylmethyl ether or styrene, or also, more especially, from vinyl chloroacetate or ethene or the like, which are well suited.

The copolymers can be made by known processes. For example, the monomer mixture of maleic anhydride and vinyl acetate in the mole ratio 1:1 may be polymerized at 80° C. in benzene solution, using peroxide catalysts, e.g. benzoyl peroxide. The reaction product precipitates in finely powdered form. If desired, there may be added to the batch, after polymerization is complete, a precipitating agent such as diethyl ether, and the polymer may be separated from the solvent by filtering. Usually no further purification is needed. The copolymers are applied to the film support in the customary manner from solutions containing 0.5 to 3.0% of the respective copolymers, and may be dried and wound up by the usual method. Film bases pretreated in this way may then be coated with a photosensitive emulsion by any of the customary methods.

By the process according to this invention the dimensional stability to processing in photographic films with

methanol 9:1 parts by volume, is treated on both sides by a prior art procedure using a substrate solution of the composition:

| Parts                                                   |
|---------------------------------------------------------|
| Vinyl acetate/maleic anhydride copolymer mole ratio 1:1 |
| Ethyl acetate                                           |
| Isopropanol                                             |

and is dried (Sample A, process according to this invention).

A second specimen of the cellulose triacetate foil designated above is treated with a substrate solution from the prior art, having the composition:

| Parts       |
|-------------|
| Gelatin     |
| Acetic acid |
| Water       |
| 55 Methanol |
| Isopropanol |
| Acetone     |

and is dried (Sample B, prior art process).

Both film supports are then coated on one side with an antihalation layer of gelatin and a suitable antihalation dye, and on the other side with a photosensitive gelatin-silver halide emulsion layer having the following properties:

|                             |              |
|-----------------------------|--------------|
| 65 AgCl:AgBr ratio          | 2:1          |
| Gelatin:silver halide ratio | 1:1          |
| Applied silver halide       | g./sq. m. 10 |

Finally the two films are developed, A and B, in a metol:hydroquinone developer of the usual composition (2 to 5 minutes, depending on the character of the developer), then fixed in a customary fixing bath (about 5 minutes), thoroughly washed and dried again.

Length measurement is effected after adequate air conditioning (20° C. and 65% relative humidity), both before

and after developing. The differences between the two measurements, which indicate the changes in film length due to the processing, are shown in the following table:

TABLE IV

|                                         | Percent change in film length<br>due to processing |            |
|-----------------------------------------|----------------------------------------------------|------------|
|                                         | Longitudinal                                       | Transverse |
| Sample A (according to this invention)- | -0.005                                             | +0.005     |
| Sample B (prior art)-----               | -0.100                                             | -0.085     |

By substituting the other specific cellulose ester film bases that are described above, similar results can be obtained.

As may be seen, the material prepared in accordance with this invention undergoes substantially no dimensional change during its processing in the photographic baths, unlike the material made with a film base treated for substrate according to the prior art.

I claim:

1. A process for making dimensionally stable organic cellulose monocarboxylic acid ester photographic film base which comprises applying to the film base an adhesive sublayer from a solution of a copolymer of one mole of maleic anhydride with one mole of a different addition polymerizable ethylenically unsaturated monomer containing a vinyl group not substituted at the  $\alpha$ -carbon atom of the vinyl group in a solvent blend of 50%-80% ethyl acetate and 50%-20% isopropanol, by weight and drying the treated film base.

2. A process according to claim 1, characterized in that a copolymer of maleic anhydride and vinyl acetate is employed.

3. A process according to claim 1, characterized in that a copolymer of maleic anhydride and vinyl chloroacetate is employed.

4. A process according to claim 1 wherein said cellulose ester is cellulose triacetate.

5. A process according to claim 1 wherein said cellulose ester is cellulose acetate/butyrate.

10

## References Cited

## UNITED STATES PATENTS

|    |           |         |                |       |            |
|----|-----------|---------|----------------|-------|------------|
| 15 | 2,067,706 | 1/1937  | Fikentscher    | ----- | 260—86.1   |
|    | 2,562,853 | 7/1951  | Baer           | ----- | 260—78.5   |
|    | 2,637,712 | 5/1953  | Upton          | ----- | 260—78.5 X |
|    | 2,756,163 | 7/1956  | Herrick et al. |       |            |
|    | 2,772,972 | 12/1956 | Herrick et al. | ----- | 96—75 X    |
|    | 3,072,482 | 1/1963  | Beeber et al.  | ----- | 96—75      |
| 20 | 3,130,051 | 4/1964  | Herrick et al. | ----- | 96—91 X    |
|    | 3,227,555 | 1/1966  | Norman         | ----- | 96—87 X    |
|    | 3,228,768 | 1/1966  | Straw et al.   | ----- | 96—75 X    |

WILLIAM D. MARTIN, Primary Examiner.

M. LUSIGNAN, Assistant Examiner.

U.S. Cl. X.R.

96—87; 117—68, 76, 83; 260—31.2, 33.4

25